

H. HAYWARD.

Paper and Process of Making the Same.

No. 226,660.

Patented April 20, 1880.



Fig. 1.



Fig. 2.



Fig. 3.



Fig. 4.

Witnesses:

Donn P. Twitchell

George Earle.



Inventor:

Henry Hayward  
By his Atts.  
Dodge Son,

# UNITED STATES PATENT OFFICE.

HENRY HAYWARD, OF NEW YORK, N. Y.

## PAPER AND PROCESS OF MAKING THE SAME.

SPECIFICATION forming part of Letters Patent No. 226,660, dated April 20, 1880.

Application filed September 30, 1879.

*To all whom it may concern:*

Be it known that I, HENRY HAYWARD, of New York, in the county of New York and State of New York, have invented certain Improvements in Paper and Processes of Making the Same, of which the following is a specification.

The object of my invention is to provide a paper which shall have great tensile strength in all directions and great flexibility combined with lightness; and to this end the invention consists in a sheet composed of paper-stock having a continuous web of long and strong fiber incorporated in its interior; and, second, in the method or process of manufacturing the same, consisting in first passing from suitable apparatus a sheet of paper-pulp, then passing from a carding or equivalent machine a continuous web of fiber tangled, crossed, and knotted together, and delivering the same into and upon the paper sheet; and, finally, delivering a layer of pulp upon the fiber, suitable suction, pressure, &c., being applied to cause a permanent and firm union or felting together of the whole in such manner as to render the same one inseparable body or sheet.

Hitherto various attempts have, I am aware, been made to combine fibrous material with paper, and among other plans attempted was that of cutting or chopping the fiber into short lengths and incorporating the same with the body of the pulp; also, that woven fabrics and prepared sheets of various kinds have been introduced between two sheets of paper and the three caused to adhere to each other; also, that fiber has been applied to the outside surface of a paper sheet, and that straight continuous lines of fiber-threads have been introduced into a paper sheet, as in the patent hitherto granted to me, and I make no claim in this patent to said methods or either of them.

Referring to the drawings, Figure 1 represents a sectional elevation of one form of apparatus for carrying out my process; Figs. 2 and 3, views showing the fiber as it appears in its original state and after passing the carding-machine, ready for introduction to the paper; Fig. 4, a sectional view of the sheet.

The apparatus used may be of any suitable character or construction, provided it is adapted to carry out my method; but that repre-

sented in the drawings is believed to be the best that can be employed.

A represents the vat containing the paper-pulp, and B a box or receiver, which receives pulp from the vat and discharges the same upon the endless wire apron of a Fourdrinier or other similar paper-machine, which may be in this regard of the ordinary and well-known construction.

D represents the slice regulating the thickness of the sheet upon the wire, as usual.

E represents an endless feeding-apron, extending from the endless wire at a point in front of the slice upward to a carding or picking machine, H, which should be of the well-known Parkhurst pattern, or of a similar character, adapted to cleanse and disentangle the fiber, split the same, if coarse, into exceedingly fine shreds, and finally deliver the same in a thin continuous web or sheet with the fibers crossed, tangled, and interlocked, as shown in Fig. 3 of the drawings.

It is particularly important that the fiber, whether hemp, jute, or other material, shall be finely divided, that it be well locked together, and that the sheet or film be comparatively thin. The sheet of pulp from the vat passes forward beneath the slice and the lower end of the apron, and receives upon its upper surface the sheet or net of fiber from the apron, which latter is so timed as to deliver the fiber at precisely the same speed as that at which the wire travels, so that the fiber is delivered quietly and smoothly into or upon the pulp without disarranging the same or destroying its continuity. Before the fiber leaves the carrier-belt E, or at the instant of its doing so, it is moistened with water or other suitable fluid by a roll, I, located beneath a water-trough. By thus dampening the fiber it is caused to unite more readily and firmly with the pulp. The sheet of pulp, with the fiber thereon, passes forward on the wire C, beneath the vat or trough J, which delivers a flow or layer of paper-pulp upon the fiber, with which and the bottom layer it readily unites. The advance of the wire carries the compound sheet over the usual suction-chamber K, which removes the surplus moisture, and beneath the dandy-roll L, and finally delivers it to the felts.

By the above process the fiber is delivered

between the two layers of pulp and the three united in one continuous indivisible sheet, which possesses great durability, strength, and flexibility. A sheet stronger than the ordinary paper can be produced with one-fourth less stock, and the expense of grinding and pulping the central fibrous portion is avoided.

The central fiber may be of any suitable kind, but, like the fiber of which the pulp is made, should be as long as possible.

Having thus described my invention, what I claim is—

1. As a new article of manufacture, the improved paper consisting of two external paper surfaces and a continuous central film or sheet of fiber crossed and tangled indiscriminately together, the whole being united in one solid indivisible sheet, as described and shown.

2. The herein-described method of manufacturing paper, consisting in producing a sheet or layer of pulp, applying a continuous webbing of crossed and tangled fiber thereon, and finally applying a second layer or film of pulp upon the fiber and uniting the whole in one sheet, as described.

3. The herein-described improvement in the art of manufacturing paper, consisting in introducing between two sheets or layers of pulp a continuous web or net-work composed of fiber crossed and entangled, as described and shown.

HENRY HAYWARD.

Witnesses:

G. W. H. ZEGLIO,  
ASHER R. MORGAN.